

Jan. 13, 1959

S. O. B. LJUNGBO

2,868,676

PRODUCTION OF NETS, KNITTED FABRICS AND THE  
LIKE FROM SYNTHETIC RESIN THREADS

Filed July 20, 1956



INVENTOR

SVEN OLOF BIRGER LJUNGBO

By Irvin S. Thompson

ATTY.

1

2,868,676

**PRODUCTION OF NETS, KNITTED FABRICS  
AND THE LIKE FROM SYNTHETIC RESIN  
THREADS**

**Sven Olof Birger Ljungbo, Stockholm, Sweden**

**Application July 20, 1956, Serial No. 599,024**

**Claims priority, application Sweden July 21, 1955**

**6 Claims. (Cl. 117—138.8)**

The present invention relates to the production of nets, knitted fabrics and the like from synthetic resin threads, and more specifically relates to an improved method of obtaining fixed knots and crossings between the threads in such nets or fabrics.

Threads made of synthetic textile material frequently involve the drawback of an excessive surface smoothness causing slippage between the threads in articles such as netting, knitted textiles, etc. in which it is desirable that the knots or crossings should be secured in a comparatively fixed interrelation.

This difficulty has been met in various ways in the past. According to certain prior methods (U. S. patent specification No. 2,590,586) the filaments are coated with a synthetic resin adapted to adhere to the filaments and being compressible to a higher degree than the latter. One drawback of this prior method is that it relies solely on such bonding action between filament and coating as is obtained by applying the coating in the form of a solution or emulsion the solvents of which are incapable of dissolving the filament or thread superficially. Where the requirements for effectiveness of the coating are higher, such as in fishing nets made of unifilar threads and required to be wetted, the bonding strength between the filament and the coating will be unsatisfactory resulting in an impaired fixation of the knots in the wetted nets.

Further prior methods (U. S. patent specification No. 2,251,508) rely on a roughening of the filament surfaces, which is accomplished by treating the filaments with a solvent for filament material and then removing this solvent, for instance by washing with a non-solvent. A similar result is obtained according to the British patent specification No. 391,480 by treating the filaments with a mixture of a solvent and a non-solvent. Both these methods result in a certain weakening of the filaments since, due to their comparatively low viscosity the solutions cannot be prevented from penetrating into the filament and causing a deep-attack thereon.

Still further prior methods are based on coating the filaments with a polymer dissolved in one or more solvents for the filament material, if desired in admixture with non-solvents, and then drying the filaments, if desired, in connection with a heat-treatment thereof. These methods, too, suffer from the drawback that the thread will be weakened due to the fact that the solutions are able to attack the same already before, through evaporation, their viscosity has been increased sufficiently to prevent deep-attacking of the threads.

In accordance with the present invention the drawbacks referred to can be overcome in the following manner:

To the thread is applied, in a manner known per se, a solution comprising a high polymer miscible with the filament material, a solvent or solvents for the filament material, and a diluent or diluents. The term "miscible

2

"with" should be understood to mean that the two polymers are incapable of precipitating the solutions of each other. The solvents should have substantially lower rates of evaporation than the diluents so that the major portion of the same remains on the threads after the diluents have evaporated. Furthermore, the solvents should be present in a sufficiently small proportion in the solution to be incapable of causing any mixing or inter-fusion of the material in the superficial layer of the thread and the high polymer applied thereto solely through the action of applying the solution and evaporating the diluent. Instead such inter-fusion or welding action is effected by heating the threads, after the evaporation of the diluent, to a sufficient high temperature to cause the polymer applied together with the remaining solvent to be transferred into a more or less liquid state. This will result in a weld between the filament surface and the polymer which, when using proper proportions of polymer and solvent, will be satisfactory without weakening the thread.

The following examples illustrate the method in a non-limitative manner:

*Example 1*

25 14 parts by weight of a co-polymerisate of methyl and butyl methacrylate  
3 parts by weight of cresol  
3 parts by weight of benzoic acid  
21 parts by weight of benzene

30 35 This solution is applied to a unifilar polyamide thread in a manner known per se so as to obtain a uniform coating on the surface of the thread. After evaporation of the benzene, the thread is subjected to heat treatment at 140° C. for a period of 30 seconds by passing the same through a chamber having this temperature. It may be suitable, in order to cause the thread to attain the proper temperature as rapidly as possible, to pass the same, immediately before or after its introduction into the heat treatment chamber, through a pool of fused metal (for instance Rose's metal) having this, or a somewhat higher, temperature, for instance 150° C. After allowing the thread to cool it may be wound on spools to be transferred to a netting process. After a net has been made of the thread, the knots therein are secured by a stretching operation in conjunction with, or subsequent to, the application thereto of a suitable solvent for the methacrylate co-polymer, for instance xylene, butyl acetate, etc. As an alternative, the net may be heated to 130 to 140° C. during the stretching operation. It is also possible to combine the two procedures.

40 45 50 It is not necessary to apply the thread coating high polymer in the form of a solution. Instead it may be applied in the form of an emulsion, the solvents for the filament material concerned being, in this case, either emulsified or dissolved in the liquid emulsifier. This is shown by the following examples:

*Example 2*

55 60 65 70 75 80 84 parts of a 50% aqueous emulsion of polybutyl methacrylate is mixed with the following suspension:

|                                    |
|------------------------------------|
| 9 parts of cresol                  |
| 9 parts of benzoic acid            |
| 0.6 part of sodium lauryl sulphate |
| 0.2 part of sodium alginate        |
| 27 parts of water                  |

The emulsion obtained is applied to a unifilar polyamide thread, and the latter is subjected to drying and further treatment in a manner similar to that of Example 1.

## Example 3

25 parts of a 40% aqueous emulsion of polymethyl methacrylate is mixed with the following suspension:

3 parts of cresol  
3 parts of benzoic acid  
0.6 part of sodium lauryl sulphate  
85 parts of water

The emulsion obtained is applied to a multifilar polyamide thread which is then subjected to further treatment in a manner similar to that of Examples 1 and 2. In spite of the fact that the polymer applied has a hardness substantially greater than that of the filament material, it is found to adhere satisfactorily to the latter as well as to result in a positive fixation of the knots in netting manufactured from such threads.

## Example 4

15% by weight of Ultramid 1C  
10% by weight of benzyl alcohol  
7% by weight of water  
68% by weight of ethanol

(Ultramid 1C is mixed polyamide of hexamethylene diamine adipate,  $\epsilon$ -caprolactam and 4,4'-diamino-dicyclohexyl methane adipate.)

The solution is used in a manner similar to that of the preceding example.

## Example 5

15% polyvinyl formal  
2% meta-acetaldehyde  
13% acetic acid  
12% benzoic acid  
58% acetone

This solution is used in a manner similar to that of the preceding examples.

The process of the present invention is illustrated in the accompanying drawing showing a flow sheet of the procedure.

What I claim is:

1. A process for treating polyamide threads and nets and knitted fabrics made therefrom with a view to obtain slip-free knots and crossings between the threads, which comprises applying to said threads, nets and knitted

fabrics a liquid composition containing at least one solvent for said polyamide, at least one liquid diluent incapable of dissolving the polyamide, and at least one polymer which is miscible with the polyamide and soluble in said solvent but insoluble in water, said solvent having a rate of evaporation which is sufficiently lower than that of said diluent to cause the major portion of the solvent applied to remain on the threads after the diluent has evaporated therefrom, the solvent being used

- 5 in a proportion which is insufficient, also after evaporation of the diluent, to effect interfusion of the polyamide of the thread and said polymer at normal temperatures, said polyamide threads, nets and knitted fabrics after evaporation of the diluent being subjected to a heat treatment whereby such interfusion is effected in the presence of the remaining solvent.
- 10 2. A process as claimed in claim 1, wherein said liquid composition is a homogeneous solution, the diluent being miscible with the solvent and the polymer being dissolved in said mixture.
- 15 3. A process as claimed in claim 1, wherein said liquid composition is a mixture of the solvent and the diluent miscible therewith, the polymer being dispersed in said liquid mixture.

- 20 4. A process as claimed in claim 1, wherein said liquid composition is a dispersion of the polymer and the solvent therefor in said diluent.

25 5. A process as claimed in claim 1, wherein the heating is effected at a temperature of from 130° C. to 150° C.

30 6. A process as claimed in claim 1, wherein the polymer is selected from the group consisting of polymethyl methacrylate, polybutyl methacrylate and co-polymerisates of methyl methacrylate and butyl methacrylate.

35

## References Cited in the file of this patent

## UNITED STATES PATENTS

- 2,251,508 Watson ----- Aug. 5, 1941  
2,590,586 Thompson et al. ----- Mar. 25, 1952  
2,639,249 Gurin et al. ----- May 19, 1953  
2,790,736 McLaughlin et al. ----- Apr. 30, 1957

## FOREIGN PATENTS

- 40 391,480 Great Britain ----- Apr. 21, 1933  
685,623 Great Britain ----- Jan. 7, 1953

45